

## UNITED STATES PATENT OFFICE

2,529,373

## TREATING SILICON STEEL

Charles H. Campbell, Bedford, and Donald S. Ferito, Cleveland, Ohio, and Carl W. Stoker, Vandergrift, Pa., assignors of one-half to The American Steel and Wire Company of New Jersey and one-half to Carnegie-Illinois Steel Corporation, both corporations of New Jersey

No Drawing. Application March 25, 1947  
Serial No. 737,086

2 Claims. (Cl. 148—12.5)

1

This invention relates to a method for improving the magnetic characteristics of silicon steels, particularly the preferred oriented silicon steels such as are used in making transformers and the like.

In the manufacture of transformer grade silicon steel strip, it is customary to anneal the strip to lower the carbon content after which the strip is again annealed to develop proper magnetic properties. We have discovered that by properly controlling the scale developed on the strip during the decarburizing anneal followed by a second anneal with a proper separating medium between the sheets or strip, that a pronounced improvement in magnetic properties is obtained.

In annealing silicon strip in conventional atmospheres, a layer of scale is formed thereon, underneath which there is formed a layer of sub-scale. The outer layer tends to be either a dense silica bearing scale which prevents proper decarburizing, or a metallic scale which causes bad surface conditions and adversely affects the magnetic properties. The sub-scale resulting from heating silicon steel in an oxidizing atmosphere is a well-defined zone of low silicon iron interspersed with particles of silica or of iron silicates. Such sub-scale is more fully described in an article entitled "Diffusion in Metal Accompanied by Phase Change," by L. S. Darken and published as Technical Publication No. 1479 by the American Institute of Mining and Metallurgical Engineers. The article appeared in the August 1942 issue of "Metals Technology." We have discovered that by proper combination of atmosphere and temperature, a layer corresponding to the structure and composition of such sub-scale can be formed directly on the surface of silicon steel sheets without any superimposed layer of scale. It has been demonstrated that the combination of a layer of scale corresponding to this sub-scale, together with box annealing with a lime separator coating is a decisive factor in achieving the desired improvement in magnetic properties.

The treatments herein disclosed may be applied to silicon steels generally, that is, electrical steels containing between .50 and 5% silicon, but is more particularly related to such steels containing between 2.5% and 3.5% silicon and which are processed so as to develop preferred grain orientation. Regular grades of silicon steel contain between .06 and .12% manganese, the manganese being reduced to such low levels because of its adverse effect on obtaining the low carbon desired, but with our treatment manganese contents of .25% or more are permissible.

Broadly the treatment consists in cold-reduc-

2

ing hot-rolled strip to the desired gauge or at least about .03 inch gauge after which it is annealed in an atmosphere and at a temperature which will give the desired scale. We have found that an atmosphere containing about 18 to 23% hydrogen, balance substantially nitrogen, the gas being saturated with water vapor at room temperature develops a satisfactory scale when the annealing temperature is between 1600° and 1725° F. Following this annealing, the strip is coated with a lime separator and given a high temperature anneal at a temperature between 1900° and 2100° F., preferably at about 2000° F. in a nitrogen atmosphere to develop the desired magnetic characteristics.

To obtain proper magnetic properties, the cold reduction is carried out in two steps. The full processing procedure for such material is as follows: silicon steel strip is hot rolled to above .08 inch gauge, pickled in acid, washed, dried, continuously cold reduced to an intermediate gauge, such as about .026 inch continuously annealed in the atmosphere controlled to develop the scale hereinbefore described, at a temperature between 1600° F. and 1725° F., using a rate of travel of about 5 feet per minute, corresponding to 5 minutes at temperature, cold reduced to the final gauge desired such as .014 inch, again continuously annealed in an atmosphere similar to the first with similar time and temperature conditions. The strip is then dipped in a lime slurry, dried, annealed at 2000° F. in an atmosphere of nitrogen. Following this, the strip may be given a stress-relief anneal by heating it for one hour at 1425° F. in a closed-muffle furnace having an atmosphere formed by keeping the residual gases in the muffle.

As before stated, we have found that an atmosphere suitable for developing the desired scale may contain 18 to 23% hydrogen, balance nitrogen, the gas being saturated with water vapor at room temperature. The gas may contain up to about 1% each of carbon monoxide and methane. The important point in connection with the gas is that it prevents the formation of a heavy silica bearing or metallic surface scale but permits a sub-scale to form directly on the surface whereby a well-defined zone of low silicon iron interspersed with particles of silica or iron silicates is built on the metal. Thus, this sub-scale is in effect a layer of steel with a reduced silicon content. Also this layer is colorless as compared to metallic scales. It is pervious to the inward passage of gas and to the outward passage of reaction gases formed by the carbon in the base metal and oxygen. Likewise, the surface is free from a heavy continuous boundary of silica

bearing scale or iron silicates, which would likewise prevent the ingress and egress of gases. As a result of this high degree of perviousness, the carbon can be lowered to the desired degree even with the higher manganese contents above noted.

To indicate the improved results from our treatment, the following data are presented. This data was obtained from sets of samples of silicon steel taken from the same coils of strip rolled and finished in the same manner with the exception that the lime coating was applied, in one case, directly on the surface of the metal, and in the other, on a layer of scale of the type herein described. This hot-rolled strip had the following composition:

|            | Per cent |
|------------|----------|
| Carbon     | .047     |
| Manganese  | .24      |
| Phosphorus | .014     |
| Sulphur    | .019     |
| Silicon    | 3.37     |

The hot-rolled strip was pickled in sulphuric acid solution until free from scale, dried and cold reduced from .08 inch to .026 inch gauge, continuously annealed by holding it at a temperature of 1675° F. for about 5 minutes in an atmosphere containing 18% hydrogen, balance substantially nitrogen and having a moisture content corresponding to a dew point of 75° F. Part of the coils were pickled to remove the scale and the others left with the scale intact. Both sets of samples were then coated with lime and box annealed at a temperature of 2000° F. in an atmosphere of nitrogen. After shearing, both sets were given a conventional stress-relief anneal for one hour at 1425° F. to relieve the shearing stresses. Tests were then made on the samples to determine the core loss as expressed in watts per pound for both 10,000 and 15,000 gausses. Column A gives the data for the samples having the scale left thereon and column B the data for those with the scale removed.

|                     | A      |        | B      |        | Per cent of Core Loss Difference |        |
|---------------------|--------|--------|--------|--------|----------------------------------|--------|
|                     | 10,000 | 15,000 | 10,000 | 15,000 | 10,000                           | 15,000 |
| 1.                  | .34    | .89    | .42    | 1.14   | 23.5                             | 28.1   |
| 2.                  | .33    | .82    | .39    | .96    | 18.1                             | 17.0   |
| 3.                  | .39    | .97    | .42    | 1.02   | 7.7                              | 5.1    |
| Difference Average. |        |        |        |        | 16.4                             | 16.7   |

This decrease of watt loss which averages over 15 per cent, greatly contributes to the quality of sheets of the above class and at the same time, the treatment does not impose any hardship or other burden on the regular processing operations.

From a theoretical standpoint, it is believed that the foregoing improvement is due to the controlled layer of scale and its behavior during the box annealing. It is generally accepted that in order to obtain proper magnetic characteristics in which a high percentage of the grains are aligned so that the 110 plane and 100 direction are in the rolling direction, it is necessary to reduce the carbon content well below .01%. It has also been generally accepted that with manganese contents greater than .15%, it is commercially impossible to lower the carbon to desired low degree and thereby permit the grains to grow in the preferred manner. However, by controlling the scale in the manner aforesaid,

carbon contents below .005% are readily obtainable in the box annealing even though the manganese content is substantially greater than .15%.

While we have shown and described one specific embodiment of our invention, it will be understood that this embodiment is merely for the purpose of illustration and description and that various other forms may be devised within the scope of our invention, as defined in the appended claims.

We claim:

1. A method of treating silicon steel containing between 2.5 and 3.5% silicon comprising continuously annealing said steel in an atmosphere containing 18 to 23% hydrogen, balance substantially nitrogen and saturated with water vapor at room temperature, the temperature of said annealing being between 1600° and 1725° F., said atmosphere and temperature combining to develop on the surface of said steel a well-defined pervious zone of low-silicon iron interspersed with silica and iron silicates, and subsequently box annealing said steel with lime in contact with the surfaces thereof in the presence of said pervious zone between 1900° and 2100° F. to further decarburize said steel and to develop the magnetic characteristics thereof.

2. A method of processing silicon steel strip, the steel thereof containing between .5 and 5% silicon comprising hot rolling said strip to above .08 inch gauge, pickling said strip to remove the scale therefrom, cold reducing said pickled strip to less than .03 inch gauge, continuously annealing said pickled strip in an atmosphere comprising between 18 and 23% hydrogen, balance substantially nitrogen and saturated with water vapor at room temperature, the temperature of said annealing being between 1600° and 1725° F., said atmosphere and temperature combining to develop on the surface of said steel a well-defined pervious zone of low-silicon iron interspersed with silica and iron silicates, and subsequently box

annealing said strip with lime in contact with the surfaces thereof in the presence of said pervious zone at a temperature of approximately 2000° F. to further decarburize said steel and to develop the magnetic characteristics thereof.

60 CHARLES H. CAMPBELL.  
DONALD S. FERITO.  
CARL W. STOKER.

#### REFERENCES CITED

65 The following references are of record in the file of this patent:

#### UNITED STATES PATENTS

| Number       | Name             | Date          |
|--------------|------------------|---------------|
| 70 886,668   | Wilks            | May 5, 1908   |
| 1,586,543    | Westberg         | June 1, 1926  |
| 2,042,124    | Reno, Jr.        | May 2, 1936   |
| 2,158,065    | Cole et al.      | May 16, 1939  |
| 2,287,467    | Carpenter et al. | June 23, 1942 |
| 75 2,307,391 | Cole et al.      | Jan. 5, 1943  |